

A. B. FOSTER,  
PROCESS OF DESULFURIZING METAL SULFIDS,  
APPLICATION FILED MAY 1, 1915.

1,296,585.

Patented Mar. 4, 1919.



Inventor  
Arthur B. Foster

# UNITED STATES PATENT OFFICE.

ARTHUR B. FOSTER, OF WASHINGTON, DISTRICT OF COLUMBIA, ASSIGNOR TO SULPHUR SYNDICATE, LIMITED, OF LONDON, ENGLAND, A CORPORATION OF GREAT BRITAIN.

## PROCESS OF DESULFURIZING METAL SULFIDS.

1,296,585.

Specification of Letters Patent.

Patented Mar. 4, 1919.

Application filed May 1, 1915. Serial No. 25,259.

To all whom it may concern:

Be it known that I, ARTHUR B. FOSTER, a citizen of the United States, residing at Washington, District of Columbia, have invented certain new and useful Improvements in Processes of Desulfurizing Metal Sulfids, of which the following is a specification.

The present invention relates to the desulfurization of metal sulfids, such as sulfid ores, and provides for the recovery, in elemental form of substantially all the sulfur content thereof. The process is applicable to such ores as contain a considerable amount of so-called "feeble atom" of sulfur, for example pyrites ores, and also to such ores as do not contain any considerable amount of feeble atom, for example pyrrhotite ore, both these ores frequently containing more or less copper, or other metal which can be recovered from the desulfurized ore, by smelting or other methods.

It has heretofore been proposed to roast ores in a reducing or non-oxidizing atmosphere, in the presence of considerable amounts of steam, to drive off the bulk of the sulfur of the ore either in the form of free sulfur or hydrogen sulfid, or mixtures of these substances, and I make no claim to such a process.

In roasting sulfid ores, particularly in the case of fine ore, it has heretofore been a common custom to roast the ore, in the presence of air, in a multiple shelf roaster, provided with rabbles, common forms of roasters for this purpose being the so-called Herreshoff furnaces, Wedge furnaces, McDougall furnaces and the like, in these operations the sulfur of the ore burning to the condition of  $\text{SO}_2$  and the iron and other metals of the ore being oxidized to the condition of oxids of these metals, which may or may not contain more or less sulfate.

It has long been recognized that hydrogen sulfid reacts with sulfur dioxid, under favorable conditions of temperature, to produce water and free sulfur, in accordance with the reaction.



This reaction has previously been utilized in various processes, having for their object the recovery of free sulfur by roasting ores.

In my process, a portion of the ore is roasted in the ordinary manner, in any suitable type of ore roasting furnace, which

may or may not be a mechanical furnace, such as one of the types of furnaces above referred to. The roasting of the ore in this manner may be accelerated if desired, by the use of solid, liquid or gaseous fuel, as has heretofore been proposed, the result of this step being the production of (a) roasted ore, consisting essentially of oxid (which may contain more or less sulfate, and usually more or less unconverted ore) and (b) gases and vapors containing considerable amounts of  $\text{SO}_2$ .

The gases and vapors are then passed, (preferably but not necessarily with the addition of more or less moisture, for example steam) through a mass or bed of unroasted ore, which may be pyrites ore, pyrrhotite ore, or the like, which mass or bed of ore is maintained at a temperature, materially above incipient redness, a temperature of 750 to 900° C. being in most instances satisfactory, but the temperature employed (when using an apparatus of the type here illustrated) will necessarily depend upon the melting point of the ore under treatment. It is not my intention to melt or sinter the ore in this step of the process, but it is preferable to maintain the ore as near the sintering temperature as is safely possible, since the reaction takes place much better at higher temperatures. It is possible, even without the addition of steam, to reduce a large part of the sulfur dioxid contained in the roaster gases to free sulfur, perhaps in accordance with the following reaction:



This reaction, or the reaction which does take place between sulfur dioxid and iron sulfid, is rather slow, at such temperature as I have been able to produce in my experiments, and accordingly I prefer to add more or less steam or moisture to the gases before passing the same into contact with the heated sulfid ore. Possibly the following reaction takes place between the steam or moisture and iron sulfid:



and the  $\text{H}_2\text{S}$  and free hydrogen thereby produced react with some of the  $\text{SO}_2$  present in accordance with reaction (1) above given. Reaction (3) goes on, at temperatures which I have been able to attain in my experiments, much more readily, and very much more completely, than reaction (2), al-

though probably all these reactions go on simultaneously.

The gases leaving the compartment, in which the ore is treated with the roaster 5 gases, will contain the major portion of the sulfur of the ore, in the form of elemental sulfur, and are then passed, preferably after suitable cooling, through any efficient type of gas washer or scrubber, such as a Feld 10 washer or the like, or any other suitable form of apparatus, for the recovery of the elemental sulfur.

In the treatment of the ore with the roaster gases, I preferably employ the ore 15 in a granular condition, which may be in the form of pieces varying in sizes from  $\frac{1}{8}$  to 1 inch. In order not to greatly impede the flow of the gases, I preferably sift out the dust-like material from this ore, before employing the same in this part of the process.

The treatment of the gases with this portion of the ore will preferably be conducted in a receptacle of considerable height, of which the lower portion is heated, in any 25 suitable manner, to the temperatures above stated, and the hot gases and vapors leaving this portion of the apparatus pass upwardly through a rather deep bed of the ore, in order to impart their heat to the incoming cooler ore. The ore treated in this 30 step may be only partially desulfurized, and may then be conveyed by suitable means into an ore roasting furnace, preferably at or near the top of the same furnace, in 35 which the other ore is roasted, or to some other furnace.

While the process forming the subject matter of my present invention may be carried out in various forms of apparatus, 40 I have shown in the annexed drawing, a form of apparatus which may be used. Said drawing shows diagrammatically, a vertical section of a suitable form of apparatus.

45 Referring to said drawing, a part of the ore is introduced through the hopper 1, into the upper compartment of an ordinary multiple shelf roaster 2 provided with suitable rabble arms 3, carrying rabbles, the 50 roasted ore being discharged through the spout 4 to a suitable conveyer 5, the rabble arms being carried by the revolving shaft 6, the ore passing downwardly over the successive hearths, 7, 8, 9, 10, 11 and 12, all in a manner well understood in the art.

To the gases and vapors leaving the roaster, through the flue 13, I may add steam through the pipe 14, the gases then entering the chamber 15, having a 60 false bottom 16 to support the bed of granular ore 17. The lower portion of this bed of ore is maintained at a temperature above incipient redness, preferably above 700° C., and I prefer to maintain the 65 ore in the bottom of this bed 17 of ore as

near the sintering point of the ore as it is possible to do, without actually sintering, a temperature of 850 to 900° C., being suitable for many kinds of ore. This heating may be accomplished in any suitable manner, electric heating being cited as one convenient mode. From this charge, ore is preferably withdrawn, either continuously or intermittently, for example by the passage 18, containing a gate 19, while fresh 75 ore is introduced through the hopper 20.

The ore introduced may be first heated to drive off any feeble atom of sulfur, but this is usually neither necessary nor desirable. The bulk of the feeble atom may be distilled 80 in the upper part of chamber 15.

To insure proper travel of the gases and vapors through the system, a pump or blower 21, or other device may be used. The gases from pipe 22 are carried off to 85 any suitable device, as above noted, for the recovery of sulfur. The reactions in the gases may not be complete until the gases and vapors reach the gas washer.

I prefer to introduce all the air for the 90 ore roasting operation at 23, but if desired a part of the air may be introduced to one or more of the compartments higher up.

In carrying out the process with such an apparatus as is here shown, the temperature 95 of the ore in the chamber 15 should preferably be kept near to, but slightly below, the temperature of incipient fusion.

What I claim is:—

1. A process of desulfurizing metal sulfids, which comprises maintaining a bed of metal sulfid, at a temperature at which iron exercises a greater affinity for oxygen than does the sulfur of sulfur dioxid, and passing gases containing sulfur dioxid through said 100 bed of metal sulfid.

2. A process of desulfurizing metal sulfids, which comprises maintaining a mass of metal sulfid, at a temperature materially above incipient redness, and maintaining 110 gases containing sulfur dioxid in intimate contact therewith, until the major part of said sulfur dioxid is reduced.

3. A process of desulfurizing which comprises roasting metal sulfid in the presence 115 of air to produce gases containing sulfur dioxid, and passing said gases in contact with a body of metal sulfid, at least a portion of which is at a temperature materially above incipient redness, while maintaining 120 contact between said gases and said metal sulfid until at least the major portion of the sulfur dioxid therein is reduced.

4. A process of treating gases containing sulfur dioxid, which comprises passing the 125 same into and through a body of metal sulfid, of which at least a part is maintained at a temperature at which the sulfur dioxid will react with the said sulfid and contacting said gases and the sulfid at the temper- 130

ature described until at least the major portion of the sulfur dioxid is reduced.

5. The improvement in the process of desulfurizing metal sulfids, which comprises treating metal sulfid, at a temperature materially above a red heat, with gases containing sulfur dioxid until at least the major portion of the sulfur dioxid is reduced.

6. A process of desulfurizing metal sulfids which comprises roasting metal sulfid to produce gases containing sulfur dioxid, treating metal sulfid, at a temperature of above 700° C., with the gases containing sulfur dioxid produced in said first 10 step until at least the major portion of the sulfur dioxid is reduced.

7. A process of desulfurizing metal sulfids which comprises roasting metal sulfid to produce gases containing sulfur dioxid, treating metal sulfid, at a temperature of above 700° C., with the gases containing sulfur dioxid produced in said first 20 step, and until at least the major portion of the sulfur dioxid of said gases is reduced, thereafter further roasting the solid product of the second step.

8. A process of desulfurizing ore which comprises contacting sulfid ore with gases containing sulfur dioxid and moisture, at a 30 temperature at which the metal of the sulfid ore has a greater affinity for oxygen than for sulfur.

9. A process of desulfurizing ore which comprises treating sulfid ore with gases containing sulfur dioxid and moisture, at a temperature materially above incipient redness until at least a material part of the sulfur dioxid is reduced.

10. A process of desulfurizing which comprises roasting metal sulfid in the presence of air to produce gases containing sulfur dioxid and passing said gases, together with moisture, into contact with a body of metal sulfid, at least a portion of which is at 40 a temperature at which the metal of the said sulfid is capable of reducing sulfur dioxid.

11. A process of treating gases containing sulfur dioxid, which comprises passing the same with moisture, into and through a 50 body of metal sulfid, of which at least a part is maintained at a temperature at which the sulfur dioxid will react with the said sulfid.

12. The improvement in the process of desulfurizing metal sulfids, which comprises treating metal sulfid with gases containing sulfur dioxid and steam at a temperature at 55 which sulfur dioxid is capable of desulfurizing said sulfid.

13. A process of desulfurizing metal sulfids which comprises roasting metal sulfid and thereby producing gases containing sulfur dioxid, maintaining contact between metal sulfid, held at a temperature of above 700° C., and gases containing steam and the

sulfur dioxid produced in said first step until at least the major portion of said sulfur dioxid is reduced.

14. A process of desulfurizing metal sulfids which comprises roasting metal sulfid 70 and thereby producing gas containing sulfur dioxid, maintaining contact between metal sulfid, held at a temperature of above 700° C., and steam and the gases containing sulfur dioxid produced in said first step, until at least the major portion of said sulfur dioxid is reduced and thereafter roasting the solid product of the second step.

15. A process which comprises passing gases containing sulfur dioxid in an upward direction through a deep bed of material containing metal sulfid, at least a part of said bed being maintained at a temperature above 700° C., while maintaining contact between said sulfid at the stated 80 temperature and said gases, until at least the major portion of the sulfur dioxid in said gases is reduced.

16. A process which comprises passing gases containing sulfur dioxid and water vapor in an upward direction through a deep bed of material containing metal sulfid, at least a part of said bed being maintained at a temperature above 700° C., while maintaining contact between said sulfid at the stated 90 temperature and said gases, until at least the major portion of the sulfur dioxid in said gases is reduced.

17. In the desulfurization of metal sulfids, the step of maintaining a bed of the 100 said sulfid at a temperature at which the metal of said sulfid exercises an affinity for oxygen greater than that exercised by sulfur for oxygen, and passing gases containing an oxid of sulfur through said bed of metal sulfid, and maintaining the said oxid of sulfur in contact with said metal sulfid until at least the major portion of the oxygen content of said oxid of sulfur combines with the metal of said metal sulfid.

18. The step of reducing sulfur oxids by maintaining persistent contact between the gases containing oxid of sulfur and a metal sulfid, at a temperature at which the metal of said sulfid has a greater affinity for the oxygen of said oxid of sulfur than for the sulfur of the metal sulfid, until at least a material amount of the oxid of sulfur is reduced.

19. The step of reducing sulfur oxids by maintaining persistent contact between the gases containing moisture and oxid of sulfur and a metal sulfid, at a temperature at which the metal of said sulfid has a greater affinity for the oxygen of said oxid of sulfur than for the sulfur of the metal sulfid, until at least a material amount of the oxid of sulfur is reduced.

20. The herein described process which comprises oxidizing the metal content of a 134

metal sulfid, by the oxygen content of an  
oxid of sulfur.

21. In desulfurizing metal sulfid the improvement which comprises maintaining a  
5 mass of solid heavy metal sulfid at a temperature at which at least one of the metals  
thereof has greater affinity for the oxygen  
of sulfur oxid than does sulfur, and bringing  
10 into contact with said sulfid, gases con-  
taining an oxid of sulfur and retaining said

metal sulfid and said gases in contact with  
each other for a sufficient time to cause the  
metal of the sulfid to unite with the oxygen  
of the sulfur and leave gases containing a  
materially less percentage of oxids of sulfur 15  
than did the gases before contact with said  
metal sulfid.

In testimony whereof I affix my signature.

ARTHUR B. FOSTER.